

Dec. 27, 1938.

H. B. BISHOP

2,141,589

LAUNDRY BLUEING AND SOURING COMPOSITION

Filed Jan. 9, 1936



WITNESS

*G. V. Rasmussen*

INVENTOR

*Howard B. Bishop*  
BY  
*Priscilla H. Bishop*  
ATTORNEYS

## UNITED STATES PATENT OFFICE

2,141,589

LAUNDRY BLUEING AND SOURING  
COMPOSITION

Howard B. Bishop, Summit, N. J.

Application January 9, 1936, Serial No. 58,272

7 Claims. (Cl. 8—77)

The present invention relates to laundry souring compositions and to an improved method of manufacturing such compositions.

The standard laundry process includes the step of washing with soap as well as a sterilizing and bleaching stage in which the fabrics are subjected to the action of sodium hypochlorite, which is alkaline in reaction. A condition of alkalinity in the cleansed and bleached fabrics would, however, cause them to become discolored and weakened in the final ironing step and it is therefore general practice to subject the cleansed laundry to souring agents. It has also been standard laundry practice to blue the cleansed fabrics to give them the desired blue-white color of properly laundered clothes.

Among the principal souring agents are acetic and oxalic acids and compounds of fluorine having an acid reaction, such as sodium acid fluoride. Among the blueing agents which have been found satisfactory are mixtures of sodium disulphonate and trisulphonate of triphenyl rosaniline. In the process of sulphonation some of the batches come out a greenish blue and some a reddish blue. By mixing a certain amount of the green with the red, a manufacturer of laundry products arrives at a standard for producing the desired shade for his requirements. These rosaniline blues, when dissolved in water or an aqueous vehicle, do not produce their full color in such liquids, but if the liquid is acidified, the blue develops.

In order to save one of the steps of the laundry process, it has heretofore been proposed to combine the blue with the sour so that the souring treatment, or at least the final part thereof, and the blueing treatment may be performed in one operation. When this was attempted in connection with sodium silico fluoride, the mixture, unless a fairly large batch of solution (containing for example approximately 10 pounds of the souring salts in 40 gallons of water with one ounce of blue dissolved in a gallon of hot water strained into it) was first made up, did not succeed in properly performing the souring operation or in adequately blueing the cloth. The reason for these results has been found by me to be due to the fact that sodium silico fluoride dissolves with difficulty and that the blue, when associated with such salts, is not uniformly distributed but tends to speck or streak the cloth. These results are in part also due to the fact that in the bleaching step of the laundry process certain parts of some fabrics, such as a turkish towel, will become over-bleached, forming oxycellulose, which has

an affinity for the blue, not only weakening the bath as a whole with respect to a uniform blue condition, but causing the blue to appear in streaks of different intensities.

The object of the present invention is to provide a laundry souring composition including a compound of fluorine having an acid reaction as the souring agent, and a blue coloring material such as an aniline blue, combined in dry dustless screened powdered form, said powder being readily soluble and being accompanied in the preferred composition by an oily coating agent. It is also an object of the invention to provide a combined souring and blueing agent which will produce uniformly treated goods without specks and streaks. Other objects of the invention will appear from the following description:

A typical method of producing my preferred composition is as follows: I place in a mixer of any suitable type, such as a rubber-lined cement mixer or a Day mixer, a major portion of crystalline ammonium silico fluoride and a minor portion of sodium silico fluoride, the proportion of the latter to the former being determined by the amount of sodium silico fluoride which will go into solution readily in a solution of the ammonium silico fluoride. A 10% aqueous solution of ammonium silico fluoride dissolves 50% more sodium silico fluoride than does pure water and by the use of ammonium silico fluoride it is possible to increase readily the amount of sodium silico fluoride in solution. To these fluorides I add about 40% by weight of anhydrous pure dextrose of the kind known on the market under the trade name "Cerelose". These three substances thus far referred to are mixed as a dry powder in a mixer, out of contact with metal, a mixing and comminuting agent being provided in the form of hard rubber balls, for example. As the mixing progresses a water solution of the blue is sprayed into the mixer. The amount of blue depends upon the grade selected for the product. For example, in regions where the water is low in alkalinity the ratio of blue to the souring agents is preferably about 1: 124. Where the water is more alkaline, the ratio is approximately 1: 160. Where the water is highly alkaline, as on the Pacific Coast, the ratio would be about 1: 200. The blue solution is made up with as little water as possible. It is preferably fed to a glass-lined vessel in amounts sufficient to make up one batch with the mixture which is being prepared in the mixer. Sulphonated castor oil dissolved for example in isopropyl ether is then fed in above the level of the blue solution.

in its glass-lined tank. About three pounds of the oil are used for 250 pounds of product. The oil floating on the blue solution is thereby positioned to enter the mixer after the last part 5 of the blue solution has been introduced to the mixer, said oil thereupon functioning to prevent dusting while the isopropyl ether, volatilizing easily, assists the oil to spread. The oil as such is without deleterious effect in the laundry process and has on the other hand a desirable, penetrating, and leveling action.

After the oil layer has been sprayed into the mixer, the procedure in the mixer is completed. The mixer is then opened, the solvent escaping, 15 the material in the mixer being run a little bit further, whereupon it is discharged into a sifter and passed through a twenty-mesh screen to remove coarse particles. Each particle of the product is by the foregoing treatment more or less 20 coated with a fine film of oil. The product dries rapidly and is non-caking. It is in crystalline or powder form and is then packed in wooden drums and shipped to the laundries for use. The laundry operator measures out his requirements 25 which are standardized for each laundry and for each kind of goods of the same general class. The powdered product, measured out as stated, is introduced to the wheel containing water and the cloth which is in readiness for the souring 30 treatment.

On the accompanying drawing is shown diagrammatically a suitable apparatus for manufacturing the souring composition described hereinabove.

A rotary mixer of conventional type is shown at 10, the same being made of rubber or other suitable material which is resistant to the action of the fluorides and other substances employed in making my improved souring composition. 40 If desired, any suitable steel or other vessel which is lined with a non-metallic resistant material may be employed, the materials being mixed out of contact with metal. Hard rubber balls (not shown) or other devices for mixing and comminuting may be employed if desired. The mixer is provided with a circumferential gear 11 which is adapted to mesh with a driving pinion (not shown) for rotating the mixer at a suitable speed. The mixer is provided with a trunnion 12 which is mounted in a pivoted bearing 13 which permits the mixer to be moved into a charging 45 position indicated in dotted lines at 1, into the operating or mixing position shown in fuel lines at 2, or into the discharging position indicated in dotted lines at 3. The capacity of the mixer is such that it holds approximately 250 pounds per unit of operation, but, of course, its capacity can be varied.

According to the grade of product which it is 60 desired to produce, a major portion of ammonium silico fluoride in crystalline form, somewhat resembling granular sugar, is introduced with an appropriate proportion of sodium silico fluoride, as much as will dissolve readily, for example, 65 in a solution of the ammonium silico fluoride. Approximately 40% by weight of anhydrous dextrose is also introduced into the mixer 10. These ingredients are mixed as dry powder in the rubber-lined cement mixer 10. The hard rubber balls tumbling about in the mixer assist in the mixing and the comminution of the particles. 70 Before adding the blue, the mixer is preferably filled with an ammonia atmosphere to neutralize any free acid in the crystals. This avoids any deleterious action on the blue.

After the ingredients of the mixer have been poured in suitable proportion into the mixer while it is in the position shown at 1, it is rotated into the full line position and the driving mechanism set into operation. One or more nozzles 14 are 5 then inserted through an opening 15 in a cover plate 16 which is attached by means of thumb screws 17 to a flange about the mouth of the mixer. The discharge opening of the nozzle is controlled by a needle valve 18 which can be 10 manually adjusted by a handle 19.

In a separate vessel or tank 20 I introduce a solution of rosaniline blue and water, using as little water as possible and using, according to the grade of product to be produced, a percentage 15 of the blue which, when mixed with the materials in the mixer 10, will give a ratio of 1 part blue to 124 parts mixture or 1 part blue to 160 parts mixture, or 1 part blue to 200 parts mixture, depending on the alkalinity of the water to be 20 employed in the souring operation or any intermediate proportions may be used. Above the level of the blue solution 21 in tank 20, I introduce the oil 21a. The vessel 20 is closed by a cover 22 which has an orifice receiving the pipe 25 23, controlled by valve 24, through which the blue solution and the oil are fed into the vessel 20 and through which subsequently air under pressure is introduced to force the contents of the vessel into the mixer 10.

The nozzle 14 may be of the type employed in spraying paint and serves for introducing the liquids in tank 20 in atomized condition into the mixed materials in the mixer. The nozzle is connected with the tank by way of a rubber hose 35 25 and a tube 26 which extends to the bottom of the tank.

Upon connecting the pipe 23 with a source (not shown) of compressed air, there is forced through the nozzle 14, first the blue solution and finally 40 the oil into the mixer, the liquids being sprayed in for purposes of thorough and uniform distribution. When the tank 20 is emptied, the nozzle 14 is withdrawn, the cover 16 of the mixer is opened, and the mixer is run a short time during which 45 the volatiles which accompanied the oil escape. Thereupon the mixer is tilted into the discharging position and the product of the mixer is passed through the sifter 27 into a car 28, said sifter being preferably a twenty-mesh screen 50 adapted to remove coarse particles.

The dextrose material acts as a leveling agent for the blue when it goes into solution in the laundry wheel and in the mixing step it takes up water, apparently forming a monohydrate of dextrose so that the mixed materials come out as a dry powder notwithstanding the introduction of the water of the blue solution.

The powdered product, which is practically dustless, is introduced into the laundry wheel 60 and the ammonium silico fluoride and sodium silico fluoride as well as the dextrose material go readily into solution, adequately souring the clothes. At the same time the blue effect is obtained and is uniform throughout the entire load, 65 probably due to the presence of the dextrose material and the sulphonated oil. The dextrose material also has an anti-color effect, killing the traces of bleach, which may still be contained in the cloth, so that as a result a brighter and clearer, more uniformly distributed blue is obtained.

According to the standard laundry process the souring step follows the rinses after the sodium hypochlorite sterilizing and bleaching stage. Then ordinarily, following the souring stage, is 75

the final blueing stage. In the present instance, where the sour and blue are combined, there is not only a saving of one operation, but there is also no such waste of sour as when the two steps 5 are separately conducted, since in the case of the new product there is an automatic check in the condition which blues with relation to the amount of sour required for the souring step, for when there is an excess of sour, the goods become 10 too blue. At the same time the result is more uniform; there is a greater snap to the color and a greater freedom from spotting and/or streaking than if the blue step were conducted as a separate operation. Furthermore, better neutralization 15 of the alkali in the cloth (higher pH in the rinse water) is obtained with the new product than with the same amount of sour without the dextrose material. Apparently the reducing action of the dextrose material converts it at least partly 20 into an organic acid which supplies additional neutralizing value.

In the new product sodium bifluoride may replace the ammonium silico fluoride though the latter is preferred. The new compound is especially adapted for use in connection with cotton fabrics.

Typical formulae giving proportions of the various ingredients used in the three different 30 grades of product hereinabove referred to are as follows:

*Dark.*—For water low in alkalinity.

|                          | Parts |
|--------------------------|-------|
| Ammonium silico fluoride | 115   |
| Sodium silico fluoride   | 25    |
| Anhydrous dextrose       | 110   |

On this is sprayed 15 parts of rosaniline blue solution containing 1 lb. dried color per gallon of water and 1½ parts sulphonated castor oil dissolved in 2½ parts of isopropylether.

*Medium.*—For water of average alkalinity.

|                          | Parts |
|--------------------------|-------|
| Ammonium silico fluoride | 159   |
| Sodium silico fluoride   | 18½   |
| Anhydrous dextrose       | 72½   |

sprayed with 10 parts blue solution containing 1 lb. dried color per gallon of water and 1½ parts sulphonated castor oil in 2½ parts of isopropyl-ether.

*Light.*—For water of high alkalinity.

|                          | Parts |
|--------------------------|-------|
| Ammonium silico fluoride | 202½  |
| Sodium silico fluoride   | 12½   |
| Anhydrous dextrose       | 35    |

sprayed with 5 parts blue solution containing 1 lb. dried blue per gallon of water and 1½ parts sulphonated castor oil in 2½ parts of isopropyl-ether. The blue calculated in the above formulae 60 is based on 100% blue content while the ordinary blue usually runs about 50%.

The rosaniline blue is a water and alcohol soluble blue wool dyestuff of single generic composition having a slightly reddish shade that will tint cotton goods to a uniform shade in a bath having a pH range from 3 to 8.5. A dilute solution of the dyestuff should have the property of being bleached to a colorless solution with either

sodium hypochlorite solution or sodium hydro-sulphite solution.

I claim:

1. A readily soluble laundry souring and bleaching composition in dry, dustless, screened, powdered form containing as its major ingredient comminuted crystalline ammonium silico fluoride, and as a minor ingredient sodium silico fluoride, said fluoride crystals being neutral with respect to free acids, and a moderately hydrated 10 anhydrous dextrose, the said crystalline components being coated with a blueing agent.

2. A readily soluble laundry souring and bleaching composition in dry, dustless, screened, powdered form containing as its major ingredient 15 comminuted crystalline ammonium silico fluoride and, as minor ingredient, sodium silico fluoride, and a moderately hydrated anhydrous dextrose, the said crystalline components being 20 coated with a blueing agent, the amount of dextrose in the composition being greater than the amount of sodium silico fluoride.

3. A readily soluble laundry souring and bleaching composition in dry, dustless, screened, powdered form containing comminuted crystalline 25 ammonium silico fluoride, sodium silico fluoride, and a moderately hydrated anhydrous dextrose, the said crystalline components being coated with a blueing agent, the proportion of sodium silico fluoride to the ammonium silico fluoride in 30 the composition being such as to go readily into solution in an aqueous solution of the ammonium silico fluoride.

4. A readily soluble laundry souring and bleaching composition in dry, dustless, screened, powdered form containing as its major ingredient 35 comminuted crystalline ammonium silico fluoride, and as a minor ingredient sodium silico fluoride, and a moderately hydrated anhydrous dextrose, the said crystalline components being 40 coated with a blueing agent, the particles of the blue-coated crystals being in turn filmed with sulphonated castor oil.

5. A composition such as set forth in claim 2, adapted for use in connection with water low in 45 alkalinity and in which the composition has approximately 115 parts ammonium silico fluoride, 25 parts sodium silico fluoride, 110 parts dextrose material, and the evaporation residues of 15 parts as blue solution containing one pound dry color 50 per gallon of water.

6. A composition such as set forth in claim 2, adapted for use in connection with water of average alkalinity and in which the composition has approximately 159 parts ammonium silico 55 fluoride, 18½ parts sodium silico fluoride, 72½ parts dextrose material, and the evaporation residues of 10 parts as blue solution containing one pound dry color of water.

7. A composition such as set forth in claim 2, adapted for use in connection with water high in alkalinity and in which the composition has approximately 202½ parts ammonium silico fluoride, 12½ parts sodium silico fluoride, 35 parts dextrose material, and the evaporation residues 65 of 5 parts as blue solution containing one pound dry color per gallon of water.

HOWARD B. BISHOP.